

April 19, 1927.

J. E. PLUMSTEAD

1,625,279

PROCESS OF UTILIZING OLD PAPER STOCK

Filed June 21, 1926



*Inventor:*

*Joseph E. Plumstead,  
by Spear, Middleton, Donahue & Hall  
Attns.*

## UNITED STATES PATENT OFFICE.

JOSEPH E. PLUMSTEAD, OF WILMINGTON, DELAWARE, ASSIGNOR TO THE JESSUP & MOORE PAPER CO., OF PHILADELPHIA, PENNSYLVANIA, A CORPORATION OF MASSACHUSETTS.

## PROCESS OF UTILIZING OLD PAPER STOCK.

Application filed June 21, 1926. Serial No. 117,483.

This invention relates to a method of producing chemically cooked pulp for use in paper making.

The invention is specifically concerned 5 with the utilization of old paper stock and paper shavings by mixing the same with new cellulosic material for the production of good pulp without the necessity of individually cooking the old paper stock.

10 To this end the invention consists in mechanically disintegrating or macerating old paper stock in water preferably made alkaline and then introducing this wet macerated mass into a tank which contains a hot charge 15 of chemically cooked pulp from a digester. The latent heat of the pulp blown from the digester has been found to be sufficient to thoroughly cook the macerated used pulp stock added thereto. The presence in this 20 blow-tank of those amounts of cooking liquor normally occurring unused in the finished charge from a digester has been found to be sufficient to de-ink and completely disintegrate the used stock so that it is then 25 in a proper condition to be bleached and finished.

I have illustrated diagrammatically in the accompanying drawing the ordinary steps taken in the treatment of chemical pulp 30 which steps are indicated in light lines and in heavy lines I have indicated the point at which this old stock is to be introduced into the system and the treatment accorded the stock before such introduction.

35 The used paper stock above referred to may be of any grade or quality depending upon the quality of pulp which it is desired to produce as an end product.

This old stock may be disintegrated in any 40 desired type of mechanical macerater.

The preliminary disintegrating process may be carried out in the cold and no heat is necessary as it is well known that heat is not essential for the disintegration of paper 45 fibres.

A hot charge from a digester is then blown into a suitable tank or receptacle to which tank has been added the macerated

stock. It has been found that in order to completely agitate and mix the two batches, 50 it is desirable to first run into the blow-tank the cold macerated stock so that the hot charge from the digester will stir the two masses as it enters the tank.

The latent heat in this hot digester charge 55 has been found sufficient to thoroughly cook the used stock and to separate the cellulosic fibres from any undesirable material contained therein. At the same time, the presence of normally occurring unused portions 60 of the cooking liquor are sufficient to de-ink and actually cook this used material.

This mixed mass is then put through the usual steps of the process leading to the production of the final pulp which includes 65 drainage and washing to free the pulp from black liquor and ink residues and the subsequent bleaching and other steps as is well known in the art.

Having thus described the invention, what 70 I claim as new is:

1. A method of cooking paper stock which consists in the step of disintegrating the same in a relatively cold state and then mixing this disintegrated stock with a hot 75 charge of chemically cooked pulp and producing finished pulp from this mixed mass.

2. A method of cooking paper stock which consists in mechanically disintegrating the same while wet and in a relatively cold state 80 in an alkaline suspension and mixing this batch with a hot charge of chemically cooked pulp.

3. A method of producing chemical pulp which consists in chemically cooking under 85 heat and pressure a charge of cellulosic containing material blowing this charge into a suitable receptacle, separately mechanically disintegrating a batch of old stock while wet and relatively cold and mixing the hot and the cold batches whereby the old stock is thoroughly cooked and the cellulosic fibres 90 separated from the undesirable material.

In testimony whereof I affix my signature.

JOSEPH E. PLUMSTEAD.